

Aug. 24, 1965

D. E. COOPER ET AL

3,201,835

## CASTING REFRACTORY METALS

Filed March 11, 1963

3 Sheets-Sheet 1



*INVENTORS.*  
Donald E. Cooper  
Schuyler A. Herres

BY

Clement Allen  
Agent

Aug. 24, 1965

D. E. COOPER ET AL.

3,201,835

## CASTING REFRACtORY METALS

Filed March 11, 1963

3 Sheets-Sheet 2



Fig. 2

*INVENTORS.*  
Donald E. Cooper  
Schuyler A. Herres

BY

  
Clement C. Cullen  
Agent

Aug. 24, 1965

D. E. COOPER ET AL

3,201,835

CASTING REFRACTORY METALS

Filed March 11, 1963

3 Sheets-Sheet 3



Fig. 5



Fig. 6



Fig. 7

INVENTORS:  
Donald E. Cooper  
Schuyler A. Herres

BY

*Donald E. Cooper*  
Agent

# United States Patent Office

3,201,835

Patented Aug. 24, 1965

1

3,201,835

## CASTING REFRACTORY METALS

Donald E. Cooper, Las Vegas, Nev., and Schuyler A. Herres, Murray Hill, N.J., assignors to Titanium Metals Corporation of America, New York, N.Y., a corporation of Delaware

Filed Mar. 11, 1963, Ser. No. 267,071

8 Claims. (Cl. 22—68)

This application is a continuation-in-part of our application Serial No. 43,205 filed July 15, 1960, now abandoned.

This invention relates to die casting of metals, and more particularly to die casting refractory metals.

Die casting has heretofore been widely used for casting relatively low melting point metals such as magnesium, zinc, aluminum, tin and lead base alloys. But the same type of machine design and process used in making die castings of such low melting point metals cannot generally be used to produce die castings of refractory metals, because such refractory metals have higher melting points and are often reactive in nature, particularly at their melting temperatures.

It is therefore an object of this invention to produce a die casting of a refractory metal. Another object of this invention is to provide a die casting machine useful for producing a casting of refractory metal. These and other objects of this invention will be apparent from the following description thereof and from the annexed drawings in which:

FIG. 1 shows a general top view of a die casting machine embodying features of this invention.

FIG. 2 shows a central vertical section of the die casting machine of FIG. 1 taken along the line 2—2.

FIG. 3 shows a front view, partly broken out, of the portion of the machine comprising the electrode actuating mechanism and the melting crucible.

FIG. 4 shows a side view, also partly broken out, of the same portion of the machine shown in FIG. 3.

FIG. 5 shows a horizontal sectional view of the portion of the machine containing the melting crucible, taken along the line 5—5 in FIG. 2.

FIG. 6 shows how the melting crucible shown in FIG. 5 is tilted in operation.

FIG. 7 shows enlarged, and in some detail, the portion of the machine comprising the injection mechanism and the die blocks.

Referring now particularly to FIGS. 1 and 2 the machine is partially enclosed in a gas tight shell indicated generally at 10 and which is composed of a bin 12, an injector housing 14, a crucible housing 16 having its top electrically insulated from the sidewalls thereof by interposition of insulating gasket 17, and an electrode housing 18. Attached to the top of electrode housing 19 preferably by removable bolts 19 (see FIG. 3) is horizontal plate 20 to which are fixedly attached vertical guide rods 22. Lower bearing plate 24 is attached to the tops of guide rods 22 and carries suitable spaced bearings 26 through which projects the tops of screw shafts 28, the lower ends of screw shafts 28 being suitably seated and maintained in similarly spaced foot bearings 30, which are attached to and carried on the upper surface of plate 20.

Spanning screw shafts 28 is lower cross head 32 which is provided with fixed nuts 34 where it is transfixed by screw shafts 28. Also attached to lower cross head 32 are spaced quick acting fluid cylinders 36 (see FIGS. 3 and 4), which may be air or hydraulic, whose piston rods 38 are fixedly attached to upper cross head 40 which is provided with suitable openings through which the screw shafts 28 pass freely. Upper cross head 40 is maintained in vertical alignment above lower cross head 32 by

2

guide rods 22, which slidably pass through suitable openings in the upper and lower cross heads 40 and 32. Fixedly attached to and depending from upper cross head 40 is electrode ram 42 which extends downwardly and passes freely through a suitable opening in lower cross head 32, and also passes through an opening in plate 20 and into electrode housing 18. An electrode, supported by the ram 42 and attached thereto at the lower end thereof by any suitable means, as by a temporary weld at 43, is shown at 44. Where ram 42 passes through plate 20, a suitable gas tight sliding seal, as at 46, is provided.

The top ends of screw shafts 28, projecting through lower bearing plate 24 are attached to pinion gears 48 which in turn mesh with central spur gear 50, suitably fixed on vertical drive shaft 52 which is journaled through an upper bearing plate 54. Bevel gear 56 is fixedly attached to the portion of drive shaft 52 which projects above upper bearing plate 54, and is in turn driven by meshed bevel gear 58 fixedly attached to the shaft 60 of electric motor 62.

Thus it will be seen that as lower cross head 32 is moved up and down by rotation of screw shafts 28, in response to actuation by motor 62 through the gear train described, upper cross head 40 will also move up and down correspondingly since the assembly of pistons 36 and piston rods 38 will ordinarily maintain the two cross heads in fixed relationship. Upper cross head 40 will thereby move electrode 44 correspondingly up and down since these elements are connected by ram 42. The direction of rotation and control of motor 62 is best accomplished by automatic means dependent on the melting arc characteristics; such means, including often an amplidyne circuit, are well known in the art and since they form no part of this invention per se, will not be described in detail. In addition to this movement control, the upper cross head 40 may be moved rapidly up and down, for reasons explained hereinafter in more detail, with respect to lower cross head 32 by action of cylinders 36, to extend or retract their piston rods 38, this being accomplished by introduction or bleeding of compressed fluid such as air through flexible hoses 64, with the air passage therethrough controlled by suitable means, such as valve 66.

Referring now particularly to FIGS. 3, 4, 5 and 6, it will be seen that electrode 44 is arranged to be lowered into or raised with respect to a cavity 68 in a crucible 70 which is provided in its top rim with indented pouring spout 72. Preferably, but not necessarily, crucible 70 is fabricated as a heavy wall body of a good heat conducting metal such as copper. It is supported inside crucible housing 16 so that it may be tilted in order for molten metal therein to be poured. This is accomplished in the embodiment illustrated by provision of saddle 74, which is generally U shaped and which is provided internally with a duct 76, through which may be circulated a cooling fluid such as water. Crucible 70 is maintained in position in saddle 74 resting on the bottom part of the U and is attached thereto as by bolts 78. Bracing members 80 are fixedly attached at their ends to the upper part of saddle 74, and encircle a top portion of crucible 70 to which they are each attached as by bolts 82. Projecting outwardly from the tops of the vertical arms of saddle 74 are hollow trunions 84 which are journaled through sealed bearings 86 in a side wall of crucible housing 16. Cooling fluid pipes 88 pass through the hollow trunions 84 extending outwardly therefrom and are preferably connected by flexible hoses 90 to a suitable source of water supply and drain, not shown.

At the exterior end of one of the hollow trunions 84 is fixedly attached crank arm 92, with its end pivotably attached, as at 94, to the piston rod 96 of air cylinder 98

which itself is suitably mounted on base plate 100, attached to an adjacent portion of the crucible housing 16 as by welded bracket 102. Compressed air is supplied through connecting hoses 104 from a source of supply, not shown, so that by appropriate action of air cylinder 98, piston rod 96 may be extended or retracted and acting through crank arm 92 and connected trunion 84, will actuate a tilting and pouring motion to crucible 70.

In the injector housing 14, and directly below the position of the pouring spout 72 in crucible 70 when the crucible is tilted to pouring position, is a funnel 106 (see FIG. 7) suitably supported by an external shell 108 which may be attached to a top member of housing 14 as by welding at 110, it being understood that an aperture is provided above funnel 106 as at 112 to allow free passage of metal poured from crucible 70. The bottom of funnel 106 leads through a short connecting pipe 114 into horizontal feed tube 116 which comprises liner 117 of graphite carried inside support steel tube 118. Slidable in feed tube 116 is closely fitting steel plunger 120 which is fixedly attached to the internal end of a plunger rod 122. Sliding seal 124 protects and maintains a gas tight passage of plunger rod 122 through the side wall of injector housing 14. The end of plunger rod 122 is connected to actuating means such as extending piston rod 126 of hydraulic cylinder 128, which itself is supported and fixedly attached to plate 130 which is attached across the outer ends of supporting bars 132 secured to the injector housing 14.

The inner end of feed tube 116 is disposed to extend through a suitable aperture in front plate 134 and is attached thereto by flange 136 which is attached to the support tube 118 as by welding, and to front plate 134 by bolts 138. Front plate 134 is suitably supported by cross brace 140 fixed between opposite sides of housing 14 and attached as by nuts 142 to the interior ends of spaced machine bars 144 which extend through the side wall of injector housing 14 and are attached at their outer ends to back plate 146. Machine bars 144 are sealed where they pass through the side wall of injector housing 14 preferably being firmly attached thereto as by welding at 148. Mounted on machine bars 144, inside the injector housing 14, is sliding plate 150, to which is attached sliding plate rod 152 which is suitably sealed with a sliding seal at 154 where it passes through the side wall of injector housing 14. The exterior end of sliding plate rod 152 is pivotably attached to toggle links 156 which in turn are pivotably attached to toggle links 158, whose exterior ends are pivotably mounted on back plate 146 as at 160. The center pivot connecting toggle links 156 and 158 is also attached at 162 to vertical link 164 which in turn is attached to the piston rod 166 of fluid cylinder 168. A suitable base plate 170 supports fluid cylinder 168 and is itself supported and connected to machine bars 144 by rods 172.

The floor of injector housing 14 is provided with an aperture 174 below the front plate 134 and sliding plate 150, and which forms a passage into bin 12. The side walls of bin 12 are preferably fabricated in two sections which may be disconnectably attached as by bolts 176 so that finished castings deposited in the bin 12 may be removed at intervals. For convenience the bin 12 is provided with supporting wheels 178.

As is customary in die casting machines the dies are split and separable. As will be seen by reference to FIG. 7, they are composed of a stationary die block 180, which is attached to front plate 134 as by bolts 182, and a movable die block 184 which is attached to sliding plate 150 as by bolts 186. It will be apparent that die blocks 180 and 184 may be separated, or locked into face-to-face relationship, by means of the mechanism previously described actuating sliding plate 150 to which movable die block 184 is attached. In the embodiment illustrated the movable die block 184 is provided with a gate 188 and runner 190 through which metal may flow into die cavity 192 formed by complimentary recesses in stationary

die block 180 and movable die block 184. It will also be seen that feed tube 116 is arranged to pass through or transfix stationary die block 180 so that it communicates with casting cavity 192 through runner 190 and gate 188.

The entire shell 10 is designed to be gas tight and provision for evacuation is made through nipple 194 which is set into and through a sidewall thereof, as shown through a sidewall of injector housing 14, and may be connected by piping 196, or other convenient means, to a vacuum pump 198 driven suitably by electric motor 200. A bleed valve 202 is arranged, as shown through a sidewall of crucible housing 16, so that air may be let into shell 10 when it is desired to break vacuum.

Power connections for supplying melting current between electrode 44 and metal in crucible 70 are arranged conveniently, as by provision of flexible cable 204 attached to cross head 40 which is in direct contact through ram 42 with electrode 44, and flexible cable 206 attached to trunion 84 which is attached and connected to saddle 74 which is in turn attached and connected to the bottom of crucible 70. Power leads 204 and 206 are connected with suitable and conventional control means to a source of high amperage electric power (not shown).

It must be realized that production of die castings of refractory and reactive metals such as titanium, zirconium, and high alloy steels, is a somewhat different operation than producing inexpensive castings of the lower melting point, and often cheaper metals. In production of die castings of zinc or aluminum, for example, rapidity of operation, volume of production and long die life are essential to profitable business. In making titanium castings, for example, the surface finish and soundness of the casting is important and the high price of the metal and limited field of usefulness would ordinarily tend to limit the number of parts required from a set of dies. The value of a finished casting would tend to make each casting a more careful and individual operation, rather than a rapid and automated output of a high volume, low price item. For this reason, it has been found that mild steel dies are quite satisfactory for the short runs most often required, and their cost, even over a short run, is not excessive in the total cost of a casting produced from a high cost metal. Over a long run period they will be subject to heat checking and corrosion; however, their original low cost, relatively easy fabrication, and lack of need of heat treating outweighs these disadvantages, which do not often become manifest during their required life.

It will be noted by those skilled in the art that the die casting machine illustrated and described herein does not contain many of the refinements and auxiliary devices at times incorporated in machines heretofore proposed and used in the making of die castings. This permits a cleaner presentation, for greater clarity and understanding of the important and unique features of the machine of this invention. It is to be understood, however, that such minor variations as employing conventional and well known parts to provide ejector pin mechanism for separating castings from a die, cores, and cooling means for dies, plates, and plunger may be incorporated if necessary or desirable.

Operation of the die casting machine of this invention will be described for illustration with reference to production of a casting of titanium metal. First the electrode housing 18 is detached from the remainder of the apparatus by loosening and removing bolts 17 and with the associated electrode control structure arranged in accessible position, the electrode ram 42 is run down by actuation of the electrode control mechanism operated by motor 62. A previously prepared electrode of titanium metal as at 44 is temporarily attached to the bottom of the electrode ram as by welding at 43, so that it may be supported in arc melting relationship to a body of refractory metal in crucible 70 when the electrode housing 18 is again assembled in operative relation with

the housing 16. A starting charge of titanium sponge or chips is placed in the bottom of crucible 70 which is adjusted into upright position by suitable actuation of air cylinder 98. With the electrode 44 now attached to the ram 42 it is run up into the electrode housing 18 and the whole electrode control assembly is replaced on top of crucible housing 16 and the bolts 17 replaced and tightened. Conveniently at this stage the electrode control cylinders 36 are actuated so that the upper cross head 40 is run down close to lower cross head 32 for reasons which will hereinafter be explained in more detail.

Suitable dies 180 and 184 with recesses to form at least one casting cavity 192, to produce the required casting are bolted in place against plate 134 and sliding plate 150 respectively. The dies are then locked together by actuation of hydraulic cylinder 168 to straighten out and align toggles 156 and 158. Plunger 120 is withdrawn to the outer end of feed tube 116 by suitable actuation of hydraulic cylinder 128, thus providing a free open passage through the funnel 106 and connecting pipe 114 into the horizontal feed tube 116. All bolts are tightened and joints checked for leaks and then the entire shell 10 is evacuated by action of vacuum pump 198.

When the pressure in the shell 10 has reached below about 5 millimeters and preferably below about 1 millimeter of mercury absolute, and it is apparent that there are no deleterious leaks in the shell, power is turned on through power leads 204 and 206 and the electrode 44 is lowered by suitable control of motor 62 operating ram 42 through the screw shafts 28 and cross head 32 until an arc is struck between the bottom end of electrode 44 and, initially, the starting charge of titanium metal in crucible 70. Following this, maintenance of the arc between electrode 44 and a pool of molten metal in crucible 70 is accomplished by suitable control of rotation of screw shafts 28 to raise or lower electrode 44, by, for example, a control unit customarily employed, based on maintenance of a uniform voltage across the arc. Under these conditions electrode 44 is progressively melted into a pool of molten titanium metal in crucible 70, with the pool being contained in a skull of solid titanium metal in contact with the inner wall of crucible 70. When the pool amounts to sufficient metal to produce the required casting together with its runners and sprue, melting power is shut off and electrode 44 is rapidly raised by actuation of cylinders 36 to lift cross head 40 with respect to cross head 32 thereby to lift the end of electrode 44 quickly out of the way of crucible 70 when tilted. Without delay, during which additional metal in the pool could be solidified in crucible 70, the crucible is quickly tilted by actuation of air cylinder 98 so that the pool of molten titanium metal in the skull inside crucible 70 is poured into funnel 106 and through tube 114 into the feed tube 116. As soon as the molten metal is received in feed tube 116, plunger 120 is, at high velocity, actuated by hydraulic cylinder 128 to force the molten metal through gate 188 and runner 190, and into the die cavity 192.

After a suitable time period to allow the casting to solidify in cavity 192, hydraulic cylinder 168 is actuated to raise central pin 162 between toggles 156 and 158, thereby to unlock and separate the die blocks by moving sliding plate 150 and its attached die away from plate 134 and the fixed die block 180. By reason of the attachment of the sprue of metal remaining in feed tube 116 and gate 188, the casting will ordinarily remain with the fixed die block 180. Plunger 120 may thereupon be again actuated inwardly by hydraulic cylinder 128 to force the casting and attached sprue and runner out of die block 180 to a position where the casting will fall by gravity into bin 12.

To produce another casting, cylinder 168 is actuated to close and lock the dies 180 and 184 together. Cylinder 128 is actuated to withdraw plunger 120 to the outer end of the feed tube 116, and crucible 70 is returned to upright

position by actuation of cylinder 98. Then cylinders 36 are actuated so that upper cross head 40 is lowered close to lower cross head 32 and this will place the electrode 44 in the cavity in crucible 70 in approximate melting position. Power between the electrode 44 and the crucible 70 is then turned on through power leads 204 and 206 and the electrode melt control system put into operation to actuate motor 62 to maintain a melting arc so that additional metal of electrode 44 is melted to form another pool or body of molten metal in crucible 70, and the steps above described are repeated.

After a suitable number of castings have been produced by a repetition of the above described cycle, which may be when all of the metal in the consumable electrode 44 has been melted into crucible 70, and the castings are sufficiently cool, the atmosphere is allowed to enter housing 10 by opening bleed valve 202. With the interior of shell 10 at atmospheric pressure, bolts 176 are then removed and the lower portion of bin 12 separated from the upper portion thereof and the finished castings removed from the bin.

Production of die castings having good surface finish and proper qualities is dependent on a number of important factors. The melting of the charged metal must be accomplished so that the molten pool in crucible 70 is enclosed in a skull of solid metal which is not so thick as to restrict the amount of metal available for pouring and casting. The heavy mass of the crucible 70 as shown and described is ideal for producing melting conditions under which a desirable pool of molten metal will be formed in side a thin skull. Fabrication of a heavy wall crucible 70 of copper will provide sufficient heat sink capacity so that the crucible itself will absorb sufficient heat during melting without the necessity for additional or external cooling. The arrangement described, in which a cooling duct 76 is provided in crucible saddle 74, makes possible the cooling of crucible 70 between pourings. It will be apparent that the heat sink capacity of the crucible 70 obviously will have a definite limit and it is a unique and valuable safety feature that the crucible itself can maintain proper operating conditions during melting without the introduction of a cooling fluid, such as water, into the furnace in this vicinity. Any leak or disruption of the cooling water system could result in contact of water with molten titanium or other reactive metal at high temperature and result in a disastrous explosion. Therefore, provision of cooling duct 76 in saddle 74, through which cooling water can be circulated at intervals when the melting operation is not in progress, enables the crucible 70 to be adequately cooled under safe operating conditions.

The metal used for die casting may be melted in crucible 70 employing either a consumable or non-consumable electrode. If consumable, the electrode 44 is fabricated of the metal to be melted and is progressively consumed and transferred into crucible 70 according to principles well known in the art. If a non-consumable electrode is employed at 44 it may conveniently be fabricated of tungsten and the metal to be melted may originally, or by suitable means be progressively charged into crucible 70 as desired. In any event, the electrode 44 is raised or lowered with respect to the metal in crucible 70 to maintain a desirable and properly operating melting arc. Control devices for accomplishing this are well known and will not herein be described in detail. They often operate in response to a signal feed back which maintains the distance between the electrode tip and the pool of molten metal so as to keep the arc voltage constant. In the case of a consumable electrode the electrode ram 42 and the electrode 44 will be gradually lowered as the electrode 44 is progressively consumed. In the case of a non-consumable electrode this may be raised or lowered but will be generally raised to maintain proper arc conditions between its tip and a gradually rising pool of molten metal in crucible 70. In any event,

at the conclusion of sufficient melting time to produce a pool composed of the required amount of metal for a single operation of the die casting mechanism, the electrode 44 must be quickly, almost instantaneously, raised so that the crucible 70 is tilted and the pool of molten metal poured therefrom. The time sequence is important since the pool of molten metal cannot be held in crucible 70, since this will result in further solidification, and an excessive amount of metal will be solidified in the skull. The electrode driving means, which in the embodiment illustrated, comprise screw shafts 28 which drive cross head 32 and cross head 40, and electrode ram 42 which supports electrode 44, and which are actuated by motor 62 through gears 48 and 50, are designed to maintain a melting arc between electrode 44 and refractory metal in crucible 70 during the melting operation. Inherently the type of mechanism involved will not be suitable for rapid or almost instantaneous movement of electrode 44. Therefore, auxiliary electrode raising means comprising fluid cylinders 36 acting on upper cross head 40 are arranged to rapidly raise ram 42 and electrode 44 independently of any position in which the cross head 32 may be situated. Thus, at the proper stage during the melting of metal in crucible 70, when it is apparent by consideration of the time of melting, or the quantity of metal melted, the power may be disconnected between electrode 44 and crucible 70, and electrode 44 raised out of the crucible cavity, and the crucible immediately tilted to pour the pool of molten metal therein into funnel 106. The sequence of these steps must be rapid and uninterrupted.

It has been found advantageous to fabricate funnel 106 of, or line it with, a suitable material, preferably one that will not react to any appreciable degree with the molten metal passing therethrough. Graphite has been found to be suitable, and the time of contact of the molten metal with the graphite funnel 106 has not been found to result in appreciable contamination of the molten metal.

The specific construction of the feed tube 116 and its cooperating plunger 120 is a key feature of this invention. As described, the feed tube 116 is fabricated with steel outer support tube 118 and a graphite liner 117. The problems in design of a workable feed tube assembly involve providing a temporary holding cylinder within which the plunger 120 can operate, the molten refractory metal in the holding cylinder being at extremely high temperature compared to the temperature when molten of metals heretofore and normally used in die casting processes. The molten metal in feed tube 116 must not be allowed to solidify, obviously, and the feed tube material must not be such as to alloy with or contaminate the refractory metal. We have found that liner 117 fabricated of graphite of a grade described in commerce as extruded graphite of good structural quality, medium grain size, pitch treated and of high bulk density, will operate advantageously inside a strong steel support tube 118. Graphite has heretofore often been proposed and used as a crucible or mold material even for castings of refractory metals. Its use in the feed tube of the die casting machine of this invention, however, becomes successful for quite different reasons; the application and purpose is quite different. Graphite in liner 117 acts as a material to maintain the molten condition of refractory metal contained therein even though its thermal conductivity is greater than adjacent or normally considered materials of construction such as steel. In a sense, graphite liner 117 acts as a thermal insulator in spite of the fact that its thermal conductivity is higher than that of steel support tube 118. Our work leads us to believe that when molten refractory metal enters feed tube 116 and contacts liner 117, the high thermal conductivity of the graphite of liner 117 results in freezing of a thin skin of solid metal around the molten metal body. Solidification of this skin results in a shrinkage of the molten

metal body which shrinks away from the graphite liner wall, thus destroying the physical contact (except perhaps along a line at the bottom) and with loss of physical contact, the overall heat transfer is substantially reduced. Additionally, graphite is characterized by a thermal capacity only about one quarter that of steel so that it actually acts to provide an initial chilling to freeze a surface skin without causing excessive heat loss from the main body of liquid metal. The thin skin of solid metal is readily rammed by the plunger 120 into the mass or "biscuit" remaining at the end of the feed tube and which is discharged attached by the sprue to the casting.

In addition, graphite resists thermal shock, is highly refractory and provides some lubricating effects when the plunger travels through it. This is probably in part the result of a wearing away of a minute amount of surface graphite with each plunger stroke. Even so and with a short contact time, the graphite liner 117 does not deleteriously contaminate the refractory metal being die cast.

The steel support tube 118 provides strength to the feed tube assembly enabling the weaker graphite liner 117 to resist the pressures and forces exerted by plunger 120.

25 The fit of plunger 120 in liner 117 is also important and the fit should be close enough so that the plunger 120 wipes the interior surface of liner 117 clean of refractory metal with each stroke. Clearance tolerance is low and should not exceed .005 inch all around. Preferably the fit between plunger 120 and liner 117 is tight and this can be obtained by making these elements of precisely mating size or fabricating the liner 117 so that its internal diameter is slightly under size with respect to the diameter of plunger 120. The first stroke of plunger 120 through liner 117 will ream out its interior to desired close fit size.

30 It will be evident that graphite liner 117 due to fit requirements and rigorous use will not be long lived. It should be replaced when clearance between its interior and plunger 120 becomes sloppy. It will, however, we have found, function efficiently for an acceptable number of ramming and casting cycles.

35 Immediately on transfer of the molten metal into the feed tube 116, plunger 120 is actuated to force the molten metal into the die cavity. Again this step must follow the previous step in rapid and uninterrupted sequence so that from the time the electrode is raised out of the cavity in crucible 70 until the plunger 120 operates to force the molten metal from feed tube 116 into the die cavities, may be of the order of only a few seconds.

40 It is necessary that operation of plunger 120 be extremely fast so that a very high velocity is imparted to the molten metal in the feed tube 116. Apparently high velocity is necessary to produce well defined and sound castings; however, extremely high pressures maintained particularly after the metal has entered the die cavities, are not necessary, as when die casting lower melting point metals, such as zinc and aluminum. Contributing to the speed and the efficiency of the complete cycle and to the quality of the castings is the fact that the shell 10, and all the melting, pouring and injecting mechanism, as well as the die blocks and die cavities, are maintained under vacuum. Thus, shell 10 forms a common chamber in which the steps of melting, pouring and forcing molten metal from the feed tube into the die cavity are carried out, with this chamber being evacuated as previously described to a pressure below about 5 millimeters of mercury absolute. This degree of vacuum will be satisfactory for producing satisfactory castings of most refractory metals. However, when casting metals such as titanium and zirconium which are in addition highly reactive, particularly with atmospheric gases at elevated temperature, the pressure in shell 10 should be preferably no greater than 1 millimeter of mercury. It will be appreciated that since the die cavities are highly evacuated

no displacement of gases occurs when molten metal is forced thereinto. Thus, the cavities forming the die cast body may rapidly be filled by molten metal forced thereinto by high velocity, and no venting of the die cavities is required; and no porosity permeated with atmospheric gases occurs in the so-produced castings. The melting, pouring and casting accomplished according to this invention under vacuum, results in a beneficial degassing of the metal employed and lack of porosity in finished castings not obtainable when such processing is carried out in the presence of appreciable amounts of atmospheric, or even inert, gases, that is above the pressures recited.

The location of bin 12 within the shell 10 provides a receptacle for holding the finished castings still under vacuum until they are sufficiently cool and ready to be exposed to the atmosphere. After casting, the metal is preferably maintained between the die blocks 130 and 134 until the formed casting has essentially solidified. At this point the die blocks may be separated and it may be removed from the die and deposited into the bin below. However, it may still be above the temperature at which exposure to air might be deleterious. Therefore, the arrangement described in the embodiment illustrated provides for cooling the finished castings to a safe temperature in an atmosphere devoid of contaminating gases to insure the best possible surface condition.

The following examples illustrate the production of die casting according to this invention.

#### Example 1

Apparatus embodying features of this invention as described hereinbefore, was employed. A 1-inch diameter tungsten inert electrode was used to melt a charge of commercially pure titanium in a heavy copper crucible using an arc current of about 2,000 amperes at about 20 volts. After a pool containing about  $\frac{1}{2}$ -pound of molten titanium had been formed in a skull of solid titanium in the crucible, the electrode was rapidly raised and the molten titanium poured into the graphite feed tube by tilting the crucible and then immediately forced by a fast acting plunger into casting cavities in a pair of mild steel die blocks. The casting cavities were in the form of specimen shapes used for tensile strength testing and were connected by runners leading to a common gate. The casting was cooled and removed from the die casting machine shell with all the above operations being carried out under vacuum of about 200 microns of mercury absolute.

The runners were removed from the cast tensile specimens. The flash at the die block parting line was ground off. The die cast specimens had a bright, smooth surface finish free from oxide or nitride contamination and were an accurate reproduction of the configuration of the cavities in which they were cast.

The die cast specimens were then pulled in a tensile testing machine and showed the following mechanical properties:

|                                 |                |
|---------------------------------|----------------|
| Ultimate tensile strength ----- | 100,000 p.s.i. |
| Yield strength (0.2%) -----     | 88,000 p.s.i.  |
| Elongation in 1 inch -----      | 20%.           |
| Reduction in area -----         | 30%.           |

Sections of the specimens showed no discernible porosity and the castings were sound and solid.

#### Example 2

The same process steps described in Example 1 were followed using the same die blocks to cast specimens of Type 316 stainless steel. Similar quality die cast tensile specimens were produced which showed the following mechanical properties:

|                                 |               |
|---------------------------------|---------------|
| Ultimate tensile strength ----- | 82,500 p.s.i. |
| Yield strength (0.2%) -----     | 42,000 p.s.i. |
| Elongation in 1 inch -----      | 63.5%.        |
| Reduction in area -----         | 70%.          |

Similar tests were performed producing the same grade and quality die castings of mild steel and A-286 (composition disclosed and claimed in U.S. Patent No. 2,641,540) alloy steel.

5 The term "refractory metal" as employed herein is intended to include those metals having a melting point above 1200° C. Such metals include titanium, zirconium, steel, alloy steels, molybdenum, tungsten, tantalum, columbium, vanadium, nickel, cobalt, as well as high melting point alloys of these metals and so-called "super-alloys." Alloys are intended to be included within the term "metal" provided they have the required high melting point to be considered refractory.

10 The die casting machine of this invention is useful for production of castings having good surface finish and sound metallurgical properties. Such castings may be suited for many applications without additional surface treatment, such as machining. The normal amount of flash resulting from the split dies as customarily employed, 15 may readily be removed by a grinding operation as is well known in the art, and separation of runner and sprue may also be accomplished by clipping, sawing or other known method of separation. The finished castings may be used 20 in applications where their form and characteristics of the metal from which they are fabricated make them particularly adapted; for example, titanium die castings may be employed in production of aircraft parts where their strength and light weight may be advantageous or they may be employed in the manufacture of marine hardware where their resistance to corrosion is a valuable 25 characteristic.

We claim:

1. In apparatus for die casting a refractory metal including a gas tight shell, a pair of separable die blocks 35 inside said shell recessed to form a casting cavity therein and means for melting a body of molten metal in a tiltable crucible in said shell the improvements which comprise;

- 40 (a) a horizontal feed tube inside said shell communicating with the casting cavity in said die blocks, said feed tube having a graphite liner,  
 (b) means for transferring molten metal from said tiltable crucible into said feed tube through the top thereof, and,  
 45 (c) a plunger inside said feed tube closely fitting the liner therein and actuated by means external of said shell to force molten refractory metal from said feed tube into the casting cavity in said die blocks.

2. Apparatus according to claim 1 in which the said feed tube has a graphite liner and an outer steel support tube.

50 3. Apparatus according to claim 1 in which the clearance between the said plunger and the said graphite liner in the feed tube does not exceed .005 inch all around.

4. Apparatus according to claim 1 in which the fit between said plunger and said feed tube is obtained by fabricating said plunger and said graphite liner of precise mating size.

5. A method for producing a die casting of a refractory metal which comprises;

- 60 (a) melting said refractory metal in a cold crucible by striking and maintaining an electric arc between an electrode and refractory metal in said crucible thereby to form a body of molten refractory metal within a skull of solidified refractory metal in said crucible,  
 (b) breaking said arc between said electrode and said molten refractory metal in said crucible when said body of molten metal in said crucible is sufficient 65 to form a die casting,  
 (c) transferring said molten refractory metal from said crucible into a graphite lined feed tube, and  
 (d) forcing said molten refractory metal from said feed tube at high velocity into a die cavity formed in metal die blocks,

(e) said steps (c) and (d) following step (b) in rapid and uninterrupted sequence thereby to prevent further solidification of said body of molten refractory metal in said crucible and to prevent deleterious solidification of said refractory metal in said feed tube and contamination of said molten refractory metal by the material of said feed tube, and steps (a), (b), (c) and (d) being carried out under vacuum.

6. A method according to claim 5 in which steps (a), (b), (c) and (d) are carried out in a common chamber evacuated to a pressure below 5 millimeters of mercury absolute.

7. A method according to claim 5 in which steps (a), (b), (c) and (d) and an additional step of cooling the so-produced die castings are carried out in a common

chamber evacuated to a pressure below 5 millimeters of mercury absolute.

8. A method according to claim 5 in which the refractory metal is titanium.

## References Cited by the Examiner

## UNITED STATES PATENTS

|           |       |                 |       |          |
|-----------|-------|-----------------|-------|----------|
| 2,610,372 | 9/52  | Schroeder       | ----- | 22—73 XR |
| 2,727,937 | 12/55 | Boyer           | ----- | 75—10    |
| 2,796,644 | 6/57  | Kuhn            | ----- | 22—69    |
| 2,799,066 | 7/57  | Federman et al. | ----- | 22—73    |
| 2,904,861 | 9/59  | Morgenstern     | ----- | 22—68 XR |
| 3,019,495 | 2/62  | Cornell         | ----- | 22—68    |

15 MARCUS U. LYONS, *Primary Examiner.*

MICHAEL V. BRINDISI, *Examiner.*